

# United States Patent Office

3,045,042

Patented July 17, 1962

1

3,045,042

# 3,045,642

## ACID POLYESTER SUCCINATES

Donald D. Staker, Nitro, W. Va., assignor to Monsanto Chemical Company, St. Louis, Mo., a corporation of Delaware  
No Drawing. Filed Aug. 16, 1957, Ser. No. 678,525  
13 Claims. (Cl. 260—485)

The present invention relates to use of chemical compounds which are oil soluble, particularly in petroleum oil fractions and which exhibit rust preventive properties towards metals, especially steel and ferrous iron surfaces. The simplest and most convenient method of developing a rust protecting film on the metal surface is to dissolve one of the preferred rust preventive compounds disclosed herein in a suitable petroleum base carrier such as motor gasoline, aviation gasoline, jet fuel, turbine oils and the like. Inasmuch as the lead salts of compounds of the preferred class of compounds do not form, or if formed are completely soluble in the petroleum fraction employed, the compounds hereinafter described may be used in leaded fuels. Thus the fuels mentioned and containing the preferred rust preventive compound may be employed as a fuel in internal combustion engines, jet engines and the like and the various parts and fittings of the engines are not damaged by deposition of insolubles and are protected from rusting. In particular fuel injection systems are not clogged or damaged by fuels containing the new adjuvants. Moreover, no insoluble alkaline earth salts are formed by reaction of sea water with the preferred class of compounds, thereby permitting the use of storage tanks previously containing a sea water ballast to be loaded with an oil fraction or a fuel treated with one of the preferred rust preventive compounds, as well as enabling storage of the treated fuel over sea water without serious loss of inhibitor taking place.

The preferred class of chemical compounds hereinafter described, and set forth as rust preventive compounds are the partial esters of an alkyl or alkenylsuccinic anhydride and preferably are the products obtained by the reaction of one molar equivalent of a polyhydric alcohol with two molar equivalents of the anhydride. Structurally the preferred class of rust preventive compounds are most conveniently represented by the formula:



wherein of the radicals R and R', one is hydrogen and the other is selected from a group comprising alkyl and alkynyl radicals preferably containing from 8 to 15 carbon atoms and R'' is the residue of the polyhydric alcohol which generically may contain oxygen, sulfur or nitrogen in the chain as well as ester substituents, and preferably contains from 3 to 6 carbon atoms. The integer n represents a number from 1 to 4 to indicate that within the purview of the invention are included the derivatives of diols, triols and other polyhydroxy compounds.

A typical procedure for the preparation of the chemical rust preventive compound employed in the present invention is the following which is illustrative only as a non-limiting procedure. The desired substituted succinic

2

anhydride and alcohol charges are weighed into a suitable jacketed acid-resisting vessel equipped with agitation, temperature recording means and a reflux condenser. The charge is heated to about 95-100° C. while agitating and held thereat and the progress of the reaction observed from time to time by withdrawing a sample and determining the neutralization number thereof. Heating is continued until the desired neutralization number is obtained or until it remains substantially constant. The reaction occurring is represented as follows:



The following are illustrative of products obtained by heating one molecular proportion of a dihydric alcohol with two molecular proportions of an alkenylsuccinic anhydride. In each case the alkenylsuccinic anhydride used was dodecenylsuccinic anhydride prepared from propylene tetramer and maleic anhydride and the product was prepared from the intermediate by heating at about 95-100° C. for the indicated times, generally without a solvent or diluent although in a few cases the reaction was carried out by heating in kerosene.

| 35 | Example | Alcohol                         | Time of Heating, hours | Neutralization Number |       |
|----|---------|---------------------------------|------------------------|-----------------------|-------|
|    |         |                                 |                        | Found                 | Calc. |
| 40 | 1       | Ethyleneglycol                  | 15.0                   | 199                   | 188.5 |
|    | 2       | Propyleneglycol                 | 23.0                   | 210                   | 184   |
|    | 3       | 1,4-Butanediol                  | 4.0                    | 181                   | 180   |
|    | 4       | 1,3-Butanediol                  | 9.0                    | 178                   | 180   |
|    | 5       | 2,3-Butanediol                  | 16.5                   | 194                   | 180   |
|    | 6       | 2-Butene-1,4-diol               | 14.0                   | 190                   | 181   |
|    | 7       | Diethyleneglycol                | 4.0                    | 183.4                 | 175   |
|    | 8       | 2,2'-Thiodiethanol              | 11.0                   | 187                   | 171   |
|    | 9       | 1,5-Pentanediol                 | 10.0                   | 184                   | 176   |
| 45 | 10      | 1,4-Pentanediol                 | 8.0                    | 189                   | 176   |
|    | 11      | Neopentylglycol                 | 15.0                   | 185                   | 176   |
|    | 12      | 1,6-Hexanediol                  | 4.0                    | 176                   | 172   |
|    | 13      | 2-Methyl-2,4-pentanediol        | 18.0                   | 250                   | 172   |
|    | 14      | Methyl-1,3-pentanediol          | 25.0                   | 187                   | 172   |
|    | 15      | Dipropylene glycol              | 9.0                    | 175                   | 168   |
|    | 16      | Triethyleneglycol               | 4.5                    | 183                   | 163   |
| 50 | 17      | 2,2,4-Trimethyl-1,3-pentanediol | 15.0                   | 165                   | 165   |
|    | 18      | 2-Ethylhexanediol-1,3           | 13.0                   | 181                   | 165   |
|    | 19      | 2,2-Diethylpropane diol-1,3     | 9.0                    | 159                   | 169   |
|    | 20      | 2,3-Dimethylhexane-2,5-diol     | 24.5                   | 271                   | 165   |
|    | 21      | Phenyl-1,2-ethandiol            | 13.5                   | 188                   | 167   |
|    | 22      | 2-Ethyl-2-butylpropane diol-1,3 | 10.0                   | 161                   | 162   |
|    | 23      | 3,6-Dimethyloctane-3,6-diol     | 18.5                   | 263                   | 158   |
|    | 24      | Polyethylene glycol 200         | 4.0                    | -----                 | 153   |
| 55 | 25      | Polyethylene glycol 400         | 4.0                    | 126                   | 121   |
|    | 26      | Polypropylene glycol 150        | 19.0                   | 179                   | 164   |
|    | 27      | Polypropylene glycol 425        | 15.0                   | 129                   | 118   |
|    | 28      | 3-Methyl-1,5-pentanediol        | 10.0                   | 174                   | 172   |
|    | 29      | Trimethylene glycol             | 11.0                   | 210                   | 184   |

60 All of the foregoing products were soluble in petroleum ether except the products from polyethylene glycol 200 and polyethylene glycol 400 which were partially soluble. The numbers following the glycol polymers indicate the molecular weight.

Using the same dodecylsuccinic anhydride as employed in the above examples, further illustrative examples are set forth below in which the ratio of the reactants varied. All these products were prepared by heating at approximately 95-105° C. for the times indicated. TPSA means tetrapropenyl (dodecyl) succinic anhydride.

| Example | Hydroxy Reactant   | Ratio of TPSA to Hydroxy Reactant | Time of Heating, Hours | Neutralization Number |       |
|---------|--------------------|-----------------------------------|------------------------|-----------------------|-------|
|         |                    |                                   |                        | Found                 | Calc. |
| 30      | 1,2,4-Butane triol | 3/1                               | 9.0                    | 191                   | 187   |
| 31      | Castor oil         | 3/1                               | 3.0                    | 107                   | 97    |
| 32      | Triethanolamine    | 3/1                               | 6.5                    | 170                   | 177   |
| 33      | Glycerol           | 2/1                               | 15.0                   | 196                   | 180   |
| 34      | Pentaerythritol    | 2/1                               | 23.0                   | 168                   | 168   |
| 35      | do                 | 4/1                               | 19.0                   | 187                   | 187   |

The various chemical products of the class described were tested to determine their solubility in petroleum oil by adding 1% by weight of the chemical product to 100 parts of petroleum ether and stirring. If any residue is observed, the product is indicated as insoluble. All of the products in the foregoing table were soluble in petroleum ether and gasoline.

In order to obtain products which do not tend to form permanent emulsions nor to precipitate alkaline earth and lead salts, the alkenyl or alkyl group is desirably within the range of 8-15 carbon atoms. However, excellent rust inhibiting properties are obtained from reactants containing alkyl and alkenyl groups outside this range. The following are illustrative of products in which the alkenylsuccinic anhydride varied. These products were prepared by heating one molecular proportion of a dihydric alcohol with two molecular proportions of the alkenylsuccinic anhydride at 95-125° C.

| Example | Alcohol                   | Anhydride | Time of Heating, Hours | Neutralization Number |       |
|---------|---------------------------|-----------|------------------------|-----------------------|-------|
|         |                           |           |                        | Found                 | Calc. |
| 36      | 2-Methyl-2,4-pentane diol | NOSA      | 28.0                   | 267                   | 208   |
| 37      | do                        | NDDSA     | 28.0                   | 224                   | 173   |
| 38      | do                        | HDSA      | 26.0                   | 192                   | 147   |
| 39      | do                        | ODSA      | 26.0                   | 170                   | 137   |
| 40      | 1,4-Butane diol           | NOSA      | 9.0                    | 225                   | 220   |
| 41      | do                        | NDDSA     | 13.0                   | 181                   | 180   |
| 42      | do                        | HDSA      | 13.0                   | 144                   | 153   |
| 43      | do                        | ODSA      | 13.0                   | 118                   | 142   |

NOSA—n-octenylsuccinic anhydride.  
NDDSA—n-dodecylsuccinic anhydride.  
HDSA—n-hexadecylsuccinic anhydride.  
ODSA—n-octadecylsuccinic anhydride.

All of the products in the foregoing table were soluble in petroleum ether except the reaction product of 1,4-butane diol and NOSA which was partially soluble.

The rust preventive properties of the chemical products were observed by carefully cleaning and polishing in the well recognized manner for performing this test on test strips of steel 3 1/2" x 5/8" x 1/16" having an S.A.E. grade designation 1020 and vigorously shaking each specimen in 75 cc. of petroleum ether containing the desired concentration or concentrations (from 5 to 20 parts per million of solvent) of the rust inhibitor. After standing for one-half hour, 2 cc. of distilled water are added and the sample is reshaken. The strip is allowed to stand in the wet petroleum ether at room temperature for about three hours, is then removed and visually inspected for rust. The results of the tests on various products of the present invention are set forth in the following table. The example numbers correspond to those

of the products identified in the foregoing tables and will serve to identify the particular material tested.

| Example | Hydroxy Reactant                 | Steel Strip Rust |           |          |
|---------|----------------------------------|------------------|-----------|----------|
|         |                                  | 20 p.p.m.        | 10 p.p.m. | 5 p.p.m. |
| 10      | Ethylene glycol                  | none             | light     | light    |
| 2       | Propylene glycol                 | trace            | none      | Do       |
| 3       | 1,4-Butane diol                  | none             | none      | none     |
| 4       | 1,3-Butane diol                  | do               | none      | Do       |
| 5       | 2,3-Butane diol                  | do               | do        | trace    |
| 6       | 2-Butene-1,4-diol                | do               | do        | none     |
| 7       | Diethylene glycol                | trace            | do        | light    |
| 8       | 2,2'-Thio diethanol              | none             | light     | light    |
| 9       | 1,5-Pentane diol                 | trace            | none      | none     |
| 15      | 1,4-Pentane diol                 | rust             | none      | light    |
| 10      | Neopentyl glycol                 | none             | none      | trace    |
| 11      | 1,6-Hexane diol                  | do               | none      | Do       |
| 12      | 2-Methyl-2,4-pentane diol        | do               | trace     | light    |
| 13      | Methyl-1,3-pentane diol          | do               | none      | Do       |
| 14      | Dipropylene glycol               | do               | none      | none     |
| 15      | Triethylene glycol               | do               | none      | rust     |
| 16      | 2,2,4-Trimethyl-1,3-pentane diol | do               | light     | none     |
| 20      | 2-Ethylhexane diol-1,3           | rust             | rust      | none     |
| 18      | 2,2-Diethylpropane diol-1,3      | none             | none      | rust     |
| 19      | 2,5-Dimethylhexane-2,5-diol      | rust             | rust      | none     |
| 20      | Phenyl-1,2-ethane diol           | none             | none      | none     |
| 21      | 2-Ethyl-2-butylpropane diol-1,3  | trace            | light     | light    |
| 22      | 3,6-Dimethyloctane-3,6-diol      | do               | rust      | rust     |
| 23      | Polyethylene glycol 200          | none             | none      | Do       |
| 24      | Polyethylene glycol 400          | do               | do        | trace    |
| 25      | Polypropylene glycol 150         | none             | light     | rust     |
| 26      | Polypropylene glycol 425         | do               | none      | Do       |
| 27      | 3-Methyl-1,5-pentane diol        | light            | rust      | none     |
| 28      | Trimethylene glycol              | none             | none      | trace    |
| 29      | 1,2,4-Butane triol               | do               | do        | light    |
| 30      | Castor oil                       | do               | do        | none     |
| 31      | Triethanolamine                  | do               | none      | Do       |
| 32      | Glycerol                         | do               | none      | Do       |
| 33      | Pentaerythritol                  | trace            | none      | Do       |
| 34      | do                               | none             | none      | Do       |
| 35      | 2-Methyl-2,4-pentane diol        | do               | none      | Do       |
| 36      | do                               | do               | none      | Do       |
| 37      | do                               | do               | do        | Do       |
| 38      | do                               | do               | do        | Do       |
| 39      | do                               | do               | do        | Do       |
| 40      | 1,4-Butane diol                  | do               | none      | Do       |
| 41      | do                               | do               | do        | light    |
| 42      | do                               | do               | do        | Do       |
| 43      | do                               | do               | do        | Do       |

Various other tests employed in the art were also utilized in the further testing of chemical products of the present invention. A description of these tests and the results obtained follow.

*Water tolerance test.*—This test is used to evaluate the emulsion characteristics of the rust inhibited petroleum fraction, such as a petroleum fuel, as set forth in A.S.T.M. D 1094-53. The apparatus consists of a 100 cc. glass stoppered graduated cylinder, which after thorough cleaning is rinsed thoroughly with distilled water and stored completely full of distilled water until used in a test. The water is removed and 80 cc. of iso-octane containing 20 parts per million of the inhibitor under test is placed in the graduate and 20 cc. of distilled water added thereto and the mixture is shaken vigorously at room temperature for 2 minutes. The mixture is then allowed to stand on a vibration-free surface for 5 minutes whereupon the volume of the aqueous layer and the amount of emulsion, if any, are recorded. In order to pass the test, the fuel shall separate sharply from the water and there shall be no evidence of an emulsion, precipitate or suspended matter within or upon either layer. Neither layer shall have changed more than 1 cc. in volume.

*Sea water reaction test.*—This test is designed to determine the solubility of the alkaline earth salts of rust inhibitors. Synthetic sea water was prepared according to the method set forth in Procedure B, A.S.T.M. D665-53T. The method consists in adding 250 cc. of n-heptane containing about 200 p.p.m. of the material to be tested and 25 cc. of synthetic sea water to a 500 cc. 3-neck flask equipped with stirrer and reflux condenser and stirring for 30 minutes at room temperature. Agitation was stopped and when motion had ceased the interface was examined for scum and the walls of the flask examined for precipitate of which there shall be none.

*Lead salt test.*—This test is designed to indicate the possibility of precipitate from the use of rust inhibitor in a

leaded gasoline. In this test, an ionizable lead salt is added to assure a concentration of lead ion. The test solution is prepared by dissolving 25 parts of lead naphthenate in 2500 parts of a regular gasoline and the solution is filtered through a double thickness of filter paper and then through a layer of fuller's earth. Thereupon 100 cc. of the test solution is added to a 500 cc. 3-neck flask equipped with a stirrer and air condenser. Agitation is started and the rust inhibitor under test is added dropwise until about 0.5 gram has been added whereupon agitation is continued for an hour at room temperature and the mixture is examined for haziness or insolubles with the aid of a flashlight. To pass the test there shall be no more haze than is exhibited by use of a blank test with no inhibitor present. The results obtained from the above-described tests are set forth in Table I wherein various reaction products of an alkenylsuccinic anhydride with the diol indicated in the table are shown.

Table I

| Example | Diol                      | Sea Water Test (insolubles) | Water Tolerance Test | Lead Salt Test (insolubles) |
|---------|---------------------------|-----------------------------|----------------------|-----------------------------|
| 3       | 1,4-Butane diol           | none                        | pass borderline      | none                        |
| 4       | 1,3-Butane diol           | do                          | do                   | do                          |
| 5       | 2,3-Butane diol           | do                          | pass                 | do                          |
| 11      | Neopentyl glycol          | trace                       | do                   | do                          |
| 12      | 1,6-Hexane diol           | do                          | do                   | do                          |
| 13      | 2-Methyl-2,4-pentane diol | none                        | do                   | do                          |
| 29      | Trimethylene glycol       | trace                       | do                   | do                          |
| 30      | 1,2,4-Butane triol        | none                        | fail                 | do                          |
| 31      | Castor oil                | trace                       | pass borderline      | do                          |
| 32      | Triethanolamine           | none                        | do                   | do                          |
| 33      | Glycerol                  | trace                       | do                   | do                          |
| 36      | 2-Methyl-2,4-pentane diol | fail                        | pass                 | trace, fail                 |
| 40      | 1,4-Butane diol           | do                          | do                   | none                        |

The rust preventing characteristics of steam turbine oil in the presence of water was determined by following A.S.T.M. Test D665-53T, Procedure B thereof. The oil employed was a base stock in commercial use for the formulation of steam turbine finished lubricants and of course contained no inhibitor of any kind. In this test, the reaction product comprising the partial ester from tetrapropenylsuccinic anhydride with the indicated diol yielded the results shown in Table II.

Table II

| Example | Diol                      | A.S.T.M. Rust Test |       |          |
|---------|---------------------------|--------------------|-------|----------|
|         |                           | 0.1%               | 0.05% | 0.03%    |
| 2       | Propylene glycol          | no rust            | light |          |
| 3       | 1,4-Butane diol           | do                 | trace | moderate |
| 5       | 2,3-Butane diol           | rust               | clean | clean    |
| 13      | 2-Methyl-2,4-pentane diol | none               | none  | light    |
| 31      | Castor oil                | rust               |       |          |
| 32      | Triethanolamine           | none               | none  | do       |
| 33      | Glycerol                  | trace              | trace | moderate |

As was shown in the reaction equation set forth illustrating the formation of the preferred rust preventive compounds, no water is evolved in the reaction of the diol and succinic anhydride derivative. The products, while containing carboxyl groups, are weak acids and do not liberate hydrogen on contact with ferrous metal or other metallic fittings used in a motor or engine. It is apparent that a wide range of products are included in the invention. Other alkenylsuccinic anhydrides have been reacted with diols as described. Thus, octenylsuccinic anhydride, dodecenylsuccinic anhydride, hexadecenylsuccinic anhydride and octadecenylsuccinic anhydride were reacted with 1,4-butane diol.

It is intended to cover all changes and modifications of the examples of the invention herein chosen for purposes

of disclosure which do not constitute departures from the spirit and scope of the invention.

What is claimed is:

1. A composition of matter soluble in petroleum oil fractions having the general formula



wherein of R and R' one is hydrogen, and the other an alkenyl radical which contains 8 to 18 carbon atoms, R'' is a residue of a polyhydric alcohol remaining from removal of  $n+1$  hydroxy groups from an alcohol containing two to four hydroxy groups attached to aliphatic carbon and  $n$  is an integer at least one but less than four.

2. A composition of matter soluble in petroleum oil fractions having the general formula



30 wherein of R and R' one is hydrogen and the other an alkenyl radical containing 8 to 15 carbon atoms, R'' is a residue of a polyhydric alcohol remaining from removal of  $n+1$  hydroxy groups from an aliphatic alcohol containing three to six carbon atoms and  $n$  is an integer at least one but less than four.

3. A composition of matter soluble in petroleum oil fractions having the general formula



wherein of R and R' one represents hydrogen and the other an alkenyl group of 8-15 carbon atoms and R'' is an alkylene group of 3-6 carbon atoms.

4. A composition of matter soluble in petroleum oil fractions having the general formula



60 wherein of R and R' one represents hydrogen and the other a branched chain dodecetyl group.

5. A composition of matter soluble in petroleum oil fractions having the general formula



wherein of R and R' one represents hydrogen and the other a branched chain dodecetyl group.

6. The process which comprises heating one mole portion of an organic polyhydroxy compound contain-

ing from 2 to 4 hydroxy radicals linked to aliphatic carbon with alkenylsuccinic anhydride the number of carbon atoms in the side chain being 8-18, the mole proportion of said anhydride being at least two, and continuing heating without formation of water until the neutralization number is essentially constant and a reaction product soluble in petroleum ether forms.

7. The process which comprises heating one mole proportion of a polyhydric alcohol containing 2-4 hydroxy radicals and two mole proportions of any alkenylsuccinic anhydride containing 8-15 carbon atoms in the alkenyl chain and continuing heating without formation of water until the neutralization number is essentially constant and a reaction product soluble in petroleum ether forms.

8. The process which comprises heating one mole proportion of a polyhydric alcohol containing 2-3 hydroxy radicals and 3-6 carbon atoms with 2-3 mole proportions of dodecenylnsuccinic anhydride, heating being continued without formation of water until the neutralization number is essentially constant and a reaction product soluble in petroleum ether forms.

9. The process which comprises heating at 95-125° C., without forming water, until the neutralization number is essentially constant two mole proportions of dodecenylnsuccinic anhydride and one mole proportion of 1,4-butane diol and a reaction product soluble in petroleum ether forms.

10. The process which comprises heating at 95-125° C., without forming water, until the neutralization number is essentially constant two mole proportions of dodecenylnsuccinic anhydride and one mole proportion of 2-methyl-2,4-pentane diol and a reaction product soluble in petroleum ether forms.

11. The process which comprises heating at 95-125°

5 C., without forming water, until the neutralization number is essentially constant two mole proportions of dodecenylnsuccinic anhydride and one mole proportion of trimethylene glycol and a reaction product soluble in petroleum ether forms.

10 12. The process which comprises heating at 95-125° C., without forming water, until the neutralization number is essentially constant three mole proportions of dodecenylnsuccinic anhydride and one mole proportion of triethanolamine and a reaction product soluble in petroleum ether forms.

15 13. A composition of matter soluble in petroleum oil fractions of the formula



wherein of R and R' one represents hydrogen and the other a branched chain dodecenyln group where N represents nitrogen.

#### References Cited in the file of this patent

#### UNITED STATES PATENTS

|    |           |                        |               |
|----|-----------|------------------------|---------------|
| 30 | 2,294,259 | Van Peski et al. ----- | Aug. 25, 1942 |
|    | 2,435,619 | Young et al. -----     | Feb. 10, 1948 |
|    | 2,442,672 | Von Fuchs et al. ----- | June 1, 1948  |
|    | 2,497,433 | Blake -----            | Feb. 14, 1950 |
|    | 2,723,286 | Young et al. -----     | Nov. 8, 1955  |
|    | 2,890,210 | Phillips et al. -----  | June 9, 1959  |